

## UNITED STATES PATENT OFFICE

2,092,529

## ALLOYS

George R. Couls, Detroit, Mich.

No Drawing. Application June 17, 1936,  
Serial No. 85,697

## 1 Claim. (Cl. 75—176)

The present invention relates to metal alloys and particularly to alloys which are largely ferrous in their composition but which contain components rendering them particularly suitable for cutting tools.

Among the objects of the invention is an alloy having the characteristics of fineness of grain, hardness, toughness, and rigidity at relatively high temperatures so as to be suitable for high speed cutting tools.

Alloys having the characteristics mentioned may be produced by fusing together and thoroughly mixing the following constituents in substantially the proportions given:

|          | Per cent     |
|----------|--------------|
| Cobalt   | 26.6 to 22.3 |
| Chromium | 27.2 to 22.8 |
| Tungsten | 22.6 to 19   |
| Iron     | 20.2 to 17   |
| Carbon   | 3.0 to 10.1  |
| Copper   | .3 to 9.23   |

or

|                       | Per cent |
|-----------------------|----------|
| Cobalt                | 26.2     |
| Ferrochromium (70-30) | 38.3     |
| Ferrotungsten (79-30) | 30.76    |
| Carbon                | 4.3      |
| Copper                | .4       |

In these two formulae the proportions and constituents are the same and the second is preferred as the ferrochrome and ferrotungsten supply the iron required, and usually part of the carbon.

While the above more or less exact proportions and constituents are preferred and produce a satisfactory product, some variation is permitted. For example, molybdenum or vanadium may be substituted for a part or all of the tungsten to produce a product which has the necessary char-

acteristics but in a lesser degree. Also a greater proportion of carbon seems to increase the hardness but at the same time makes the product more brittle. If, however, when increasing the carbon content, the copper is also increased, some of the brittleness is prevented.

In making the alloy it is preferred to fuse together all of the constituents except the copper and to thoroughly mix, then to add the copper. If desired, the melt may be made of the constituents without the copper and allowed to set. This, however, must be remelted and the copper added to produce a product having the desirable properties. After the addition of the copper the mass should be maintained in the molten condition for a short period to permit the copper to exert its action upon the mixed constituents. The copper seems to toughen the resulting product.

When making the copper addition, it is preferred to mix the copper in the melt and allow the mass to stand for a short period in the molten condition to permit the copper to exert its action. The copper appears to exert upon the alloy constituents some sort of modifying action, the exact nature of which is not clear. The procedure however, produces a better product than if the casting operation follows immediately the copper addition.

What I claim is:

An alloy consisting of the following constituents in approximately the proportions stated:

|          | Per cent     |
|----------|--------------|
| Cobalt   | 22.6 to 22.3 |
| Chromium | 27.2 to 22.8 |
| Tungsten | 22.6 to 19   |
| Iron     | 20.2 to 17   |
| Carbon   | about 4.5    |
| Copper   | about 1      |

GEORGE R. COULS.